

1

3,376,207

## ELECTRODEPOSITION OF NICKEL AND ELECTROLYTES THEREFOR

Harry Axel Herman Ericson, Warby, Fittja, Sweden, assignor to Patent-Serm AG., Lucerne, Switzerland, a firm

No Drawing. Filed May 17, 1965, Ser. No. 456,541  
26 Claims. (Cl. 204—49)

The present invention relates to the electrodeposition of nickel from an aqueous acidic nickel plating bath and, more particularly, to the production of bright and level electrodeposits of good ductility and adherence.

It is known to modify nickel electroplating baths with brightening agents as well as with agents to improve leveling effects. However, it has been observed that during the electroplating process when the bath contains conventional brightening and leveling agents, hydrogen is evolved at the cathode in quantities sufficient to produce deleterious effects which result in reduced corrosion protection for the base metal.

It is, therefore, an object of this invention to provide an electroplating process whereby bright, level and adherent nickel electrodeposits can be obtained free from the disadvantageous effects of hydrogen evolution at the cathode which substantially reduces the corrosion protection desired for the base metal.

Another object of this invention is to provide an additive for nickel plating baths from which bright, level, ductile and adherent nickel deposits may be obtained.

A further object of this invention is to provide an additive for nickel plating baths which is employed to reduce the evolution of hydrogen at the cathode so as to produce on the base metal a porous-free deposit having increased corrosion protection characteristics.

With the foregoing objects in view, as well as others which will become apparent as the description proceeds, the invention consists in the novel plating process, the novel additive and bath compositions which will be described in certain illustrative examples hereinafter and which will then be more particularly pointed out in the appended claims.

It has now proved possible to produce nickel coatings with high brightness and good ductility by employing nickel plating baths containing a brightener selected from the group of compounds having the following structural formula:



wherein R, R<sub>1</sub>, R<sub>2</sub> and R<sub>3</sub> are selected from the group consisting of hydrogen, alkanyl, alkenyl, alkynyl, the hydroxy derivatives of said alkanyl, alkenyl and alkynyl radicals, amino and sulfonic acid groups, and X is halogen. Preferably, the alkanyl, alkenyl and alkynyl radicals have 1-6 carbon atoms.

Representative sulfonylethers having the structural formula



include methyl sulfonylether, ethyl sulfonylether, hydroxyethylene sulfonylether, butyl sulfonylether, propyl sulfonylether, hydroxybutylene sulfonylether, vinyl sulfonylether, 1-propenyl sulfonylether, 2-pro-

2

penyl sulfonylether, isopropenyl sulfonylether, 1-butenyl sulfonylether, 2-butenyl sulfonylether, hydroxybutenyl sulfonylether, propargyl sulfonylether, 1-butyneyl sulfonylether, 2-butyneyl sulfonylether, 1-pentyneyl sulfonylether, 4-hydroxy-2-butyneyl sulfonylether, aminoethylene sulfonylether, 2-propenylaminoethylene, sulfonylether, propargylaminoethylene sulfonylether, sodium sulfonate sulfonylether, sodium ethylenesulfonate sulfonylether.

10 Representative aminosulfolanes having the structural formula



15 include methylamino sulfolane, 2-propenylamino sulfolane, propargylamino sulfolane, N<sup>1</sup>-propargylamino, N<sup>2</sup>-ethyleneamino sulfolane, sodium sulfonamyl taurate, dihydroxydiethyleneamino sulfolane, N-hydroxyethylene N-2-propenylamino sulfolane, N-hydroxyethylene-N-propargylamino sulfolane, N-butyl, N-propargylamino sulfolane, N<sup>1</sup>-propargylamino, N<sup>2</sup>-butyl-N<sup>2</sup>-ethyleneamino sulfolane, sodium sulfonamylmethyl taurate, dipropenylamino sulfolane, N-propenyl-N-propargylamino sulfolane, sodium sulfonamylpropenyl taurate, dipropargylamino sulfolane, N<sup>1</sup>-propargylamino, N<sup>2</sup>-propargyl-N<sup>2</sup>-ethyleneamino sulfolane, sodium sulfonamylpropargyl taurate, di-N<sup>1</sup>-propargylamino, N<sup>2</sup>-ethyleneamino sulfolane, sodium sulfonamyl, N<sup>1</sup>-propargylamino, N<sup>2</sup>-ethyleneamino taurate, di-sodium sulfonamylpropargyl taurate, tetraamino tetraethylene aminosulfolane, propargylamino-triamino-tetraethylene aminosulfolane, propargylamino-diamino-triethylene aminosulfolane, and propargylamino-monoamino-diethylene aminosulfolane.

20 Representative preferred sulfonylesters having the structural formula



25 include acetyl sulfonylester chloride, acryl sulfonylester chloride. It has also been found 3-sulfolanol can also be advantageously employed as well as 3-sulfolene which has the power to act as a source of sulfur dioxide. 3-sulfolene decomposes in sulfur dioxide and butadiene. At 70° C. the decomposition rate is approximately 0.1% per hour. In situations where hexavalent chromium is present or where exceptionally good throwing or covering power is desired sulfolene is an excellent addition agent to the aqueous acidic nickel plating bath.

30 The novel brighteners of this invention are generally used in amounts between 0.01 and 10 millimoles per liter of bath solution and preferably between 0.02 to 1.0 millimole per liter of solution.

35 In general, the process of the invention involves operating a bath at conventional nickel plating temperatures ranging from about 30° C. to as high as 80° C. with a range of 40-65° C. being especially desirable. The pH of the plating bath, as determined electrochemically, can range from around 1.5 to 5.0 with 3.0 to 5.0 being found especially suitable in the majority of cases. Practically all baths for electroplating nickel contain nickel sulfate, a chloride, usually nickel chloride, a buffering agent, usually boric acid and a wetting agent. Such types of baths include the well-known Watts-type bath and high chloride type bath. The Watts bath solution to which the

novel brightener of this invention can be added typically comprises around 300 grams per liter of nickel sulfate, 60 grams per liter of nickel chloride and 40 grams per liter of boric acid. The foregoing bath composition and specified operating conditions are not critical in the basic Watts bath solution and the particular temperature and pH thereof may vary within the indicated ranges without adverse effects. Considerable latitude is also permissible in respect to the types and concentrations of the nickel salts employed, for instance, as the source of nickel, a combination of nickel fluoborate with nickel sulfate and nickel chloride, or a combination of nickel fluoborate with nickel chloride can be used.

In another embodiment of this invention the nickel plating bath solution can contain, in addition to the novel brightener of this invention, a brightener of the first class which is, preferably, an aromatic sulfur compound such as p-toluene sulfonamide, o-benzoyl sulfimide, benzene sulfonamide, naphthalene tri-sulfonic acid, benzene sulfonic acid, 2-butyne, 1,4-disulphonic acid, allyl sulfonic acid together with 2-butyne, 1,4-dioxyethanesulfonic acid or sodium saccharate. Generally the aromatic sulfur compound will be present in amounts ranging from 0.1 to 30 grams per liter of solution. Additionally, if the bath is air agitated, comparable brightening effects are obtained with a substantially less brightener concentration. In this latter instance the novel brightener of the invention is generally employed in amounts ranging between 0.025 to 2.5 millimoles per liter of solution while the brightener of the first class advantageously is employed in amounts ranging from 0.05 to 15 grams per liter of solution. A mirror bright deposit of high luster is obtained when using this combination of brighteners especially when the novel brightener of this invention is an unsaturated aminosulfolane.

Various wetting agents can be used in association with the novel plating bath compositions of this invention such as sodium lauryl sulfate, sodium lauryl ether sulfate and 7-ethyl-2-methyl-4 undecanol. Further, wetting agents which can be used have the following formula and are used in amounts of 0.5 to 5 grams per liter:



wherein  $R_4$  is an alkanoyl group having 8 to 10 carbon atoms,  $R_5$  is selected from the group consisting of hydrogen, aliphatic, alicyclic and aromatic radicals,  $R_6$  is an aliphatic bridge containing from 1 to 5 carbon atoms and  $R_7$  is selected from the group consisting of hydrogen and alkali metals. Representative wetting agents of this type are sodium octanoyl taurate, potassium nonanoyl methyl taurate, sodium decanoyl methyl taurate, sodium octanoyl cyclohexyl taurate, sodium nonanoyl methyl phenyl taurate, sodium decanoyl phenyl taurate, sodium octanoyl cyclopropyl taurate, octanoyl hexyl amino propylene sulfonic acid, sodium salt of decanoyl cyclobutyl amino butylene sulfonic acid, and octanoyl tauric acid.

To reduce the sensitivity of the novel nickel plating bath compositions of this invention with respect to metallic and/or organic contaminants, a hydroxy derivative of an aromatic sulfur compound such as sodium tetrahydroxynaphthalene sulfonic acid can be added to the bath solution as a sequestering agent. Preferably, the sequestering agent is employed in amounts of 0.1 to 5 grams per liter of plating solution.

For the purpose of giving those skilled in the art a better understanding of the invention, illustrative examples are given. In the examples, an aqueous acidic nickel-containing bath was made up with the specified components. Electrodeposition was carried out by passing electric current through an electric circuit comprising an anode and a sheet metal or rod cathode, both immersed in the bath. The baths were agitated, usually by a moving cathode although in certain instances air agitation was employed. The examples utilizing the novel brighteners of this invention resulted in a nickel coating with improved leveling effects and corrosion resistance properties. In the examples employing, additionally, a brightener of the first class, i.e. an aromatic sulfur compound, the resulting sulfur-containing nickel coating also exhibited mirror bright characteristics as well as stress-free properties.

In the examples, the following standard Watts-type bath was used as a base solution:

|    |                 |       |         |
|----|-----------------|-------|---------|
| 10 | Nickel sulfate  | g./l. | 300     |
|    | Nickel chloride | g./l. | 60      |
|    | Boric acid      | g./l. | 40      |
|    | pH              |       | 3.0-5.0 |
| 15 | Temperature     | ° C.  | 40-60   |

#### EXAMPLE 1

|    |                           |                          |      |
|----|---------------------------|--------------------------|------|
| 20 | Propargyl sulfolanylether | mmol/l.                  | 0.3  |
|    | Sodium saacharate         | g./l.                    | 1.5  |
|    | Sodium lauryl sulfate     | g./l.                    | 0.1  |
|    | Current density           | amperes/dm. <sup>2</sup> | 1-10 |

#### EXAMPLE 2

|    |                                |                          |      |
|----|--------------------------------|--------------------------|------|
| 25 | Hydroxybutynyl sulfolanylether | mmol/l.                  | 0.1  |
|    | Sodium saccharate              | g./l.                    | 1.5  |
|    | Sodium lauryl sulfate          | g./l.                    | 0.1  |
|    | Current density                | amperes/dm. <sup>2</sup> | 1-10 |

#### EXAMPLE 3

|    |                                              |                          |      |
|----|----------------------------------------------|--------------------------|------|
| 30 | 1-butenyl sulfolanylether                    | mmol/l.                  | 0.5  |
|    | Sodium saccharate                            | g./l.                    | 1.0  |
|    | Sodium tetrahydroxynaphthalene sulfonic acid | g./l.                    | 1.0  |
|    | Current density                              | amperes/dm. <sup>2</sup> | 2-15 |

#### EXAMPLE 4

|    |                                                  |                          |      |
|----|--------------------------------------------------|--------------------------|------|
| 40 | Sodium hydroxyethylene-N-propargylaminosulfolane | mmol/l.                  | 0.5  |
|    | Sodium saccharate                                | g./l.                    | 1.5  |
|    | Sodium oleinoylmethyl taurate                    | g./l.                    | 0.1  |
|    | Current density                                  | amperes/dm. <sup>2</sup> | 1-10 |

#### EXAMPLE 5

|    |                                              |                          |      |
|----|----------------------------------------------|--------------------------|------|
| 45 | Propargyl sulfolanylether                    | mmol/l.                  | 0.6  |
|    | Naphthalene trisulfonic acid                 | g./l.                    | 10   |
| 50 | Sodium tetrahydroxynaphthalene sulfonic acid | g./l.                    | 1    |
|    | Sodium sulfolanylmethyl taurate              | mmol/l.                  | 1    |
|    | Current density                              | amperes/dm. <sup>2</sup> | 2-15 |

#### EXAMPLE 6

|    |                                    |                          |      |
|----|------------------------------------|--------------------------|------|
| 55 | Sodium sulfolanylpropargyl taurate | mmol/l.                  | 0.5  |
|    | Sodium saccharate                  | g./l.                    | 1.5  |
|    | Sodium octanoyl taurate            | g./l.                    | 0.1  |
|    | Current density                    | amperes/dm. <sup>2</sup> | 2-15 |

#### EXAMPLE 7

|    |                                              |                          |      |
|----|----------------------------------------------|--------------------------|------|
| 60 | 2-propenyl sulfolanylether                   | mmol/l.                  | 10   |
|    | Sodium saccharate                            | g./l.                    | 1.5  |
|    | Sodium tetrahydroxynaphthalene sulfonic acid | g./l.                    | 1    |
|    | Current density                              | amperes/dm. <sup>2</sup> | 1-10 |

#### EXAMPLE 8

|    |                                              |                          |      |
|----|----------------------------------------------|--------------------------|------|
| 70 | 2-butenyl sulfolanylether                    | mmol/l.                  | 0.1  |
|    | Sodium tetrahydroxynaphthalene sulfonic acid | g./l.                    | 1    |
|    | Current density                              | amperes/dm. <sup>2</sup> | 1-10 |

## EXAMPLE 9

2-butynyl sulfolanylether mmol/l... 5  
 Current density amperes/dm.<sup>2</sup> 2-15

## EXAMPLE 10

1-hydroxybutenyl sulfolanylether mmol/l... 0.5  
 Current density amperes/dm.<sup>2</sup> 2-15

## EXAMPLE 11

1-hydroxy 2-butynyl sulfolanylether mmol/l... 0.7  
 Sodium saccharate g./l... 1.5  
 Sodium octanoyl cyclohexyl taurate g./l... 1  
 Current density amperes/dm.<sup>2</sup> 1-10

## EXAMPLE 12

Dihydroxydiethylenecamino sulfolane mmol/l... 1  
 Current density amperes/dm.<sup>2</sup> 1-10

## EXAMPLE 13

Ethanolamino sulfolane mmol/l... 5  
 Sodium saccharate g./l... 1  
 Current density amperes/dm.<sup>2</sup> 2-15

## EXAMPLE 14

N-hydroxyethylene-N-propargylamino sulfolane mmol/l... 1  
 p-toluene sulfonamide g./l... 10  
 Current density amperes/dm.<sup>2</sup> 1-10

## EXAMPLE 15

N-butyl-N-propargylamino sulfolane mmol/l... 0.10  
 Sodium lauryl sulfate g./l... 0.1  
 Current density amperes/dm.<sup>2</sup> 1-10

## EXAMPLE 16

2-propenylamino sulfolane mmol/l... 5  
 Sodium tetrahydroxynaphthalene sulfonic acid g./l... 1  
 Current density amperes/dm.<sup>2</sup> 2-15

## EXAMPLE 17

N-hydroxyethylene-N-2-propenylamino sulfolane mmol/l... 5  
 Sodium lauryl sulfate g./l... 1  
 Current density amperes/dm.<sup>2</sup> 2-15

## EXAMPLE 18

Butyl-N-propargylamino sulfolane mmol/l... 0.1  
 Current density amperes/dm.<sup>2</sup> 2-5

## EXAMPLE 19

3-sulfolanol mmol/l... 5  
 Sodium saccharate g./l... 1  
 Current density amperes/dm.<sup>2</sup> 2-15

## EXAMPLE 20

N'-propargylamino N<sup>2</sup>-ethylenecamino sulfolane mmol/l... 1  
 Sodium saccharate g./l... 1  
 Current density amperes/dm.<sup>2</sup> 1-10

## EXAMPLE 21

Sodium sulfolanyl taurate (Sulfolanyl-aminoethylene sulfonic acid, sodium salt) mmol/l... 5  
 Current density amperes/dm.<sup>2</sup> 1-10

## EXAMPLE 22

Sodium sulfolanylmethyl taurate (Sulfolanyl-amino-methyl N-ethylene sulfonic acid, sodium salt) mmol/l... 1  
 10 Sodium saccharate g./l... 1  
 Current density amperes/dm.<sup>2</sup> 1-10

## EXAMPLE 23

Sodium sulfolanyl propargyl taurate mmol/l... 10  
 Current density amperes/dm.<sup>2</sup> 1-10

## EXAMPLE 24

Acryl sulfolanylester chloride mmol/l... 1  
 Sodium saccharate g./l... 1  
 Current density amperes/dm.<sup>2</sup> 2-15

## EXAMPLE 25

Tetraamino-tetraethylene aminosulfolane mmol/l... 0.02  
 Naphthalene trisulfonic acid, sodium salt g./l... 5.0  
 30 Sodium saccharate g./l... 0.5  
 Sodium laurylsulfate g./l... 0.1

## EXAMPLE 26

Propargylamino - triamino - tetraethylene aminosulfolane mmol/l... 0.01  
 Sodium saccharate g./l... 0.5  
 Sodium laurylsulfate g./l... 0.1

## EXAMPLE 27

Propargylamino - diamino - triethylene aminosulfolane mmol/l... 0.02  
 Sodium saccharate g./l... 0.5  
 Sodium laurylsulfate g./l... 0.1

## EXAMPLE 28

Propargylamino - amino-diethylene aminosulfolane mmol/l... 0.02  
 50 Sodium saccharate g./l... 0.5  
 Sodium laurylsulfate g./l... 0.1

The novel sulfolene brighteners of the instant invention can also be used in combination with any of the conventional brighteners of the second class (levelers). Synergistic effects have been noted as illustrated in the following example.

## EXAMPLE 29

Tetraamino-tetraethylene aminosulfolane mmol/l... 0.02  
 Bis-hydroxyethyl ether of butynediol g./l... 0.025  
 Sodium saccharate g./l... 0.5  
 60 Sodium laurylsulfate g./l... 0.1

Unless otherwise specified all parts and percentages in the specification and claims are by weight. The foregoing examples illustrate specific baths and processes, several being preferred. It is to be understood that the compositions and conditions can be varied. Therefore as many embodiments of this invention may be made without departing from the spirit and scope thereof and the invention includes all such modifications and variations as come within the scope of the appended claims.

What is claimed is:

1. An aqueous acid bath solution for electroplating nickel containing at least one nickel salt as a source of nickel which plating solution includes as brightener a sufficient amount of a compound selected from the group consisting of compounds having the structural formula



10

and



wherein R, R<sub>1</sub>, R<sub>2</sub> and R<sub>3</sub> are selected from the group consisting of hydrogen, alkanyl, alkenyl and alkynyl radicals, hydroxy derivatives of said alkanyl, alkenyl and alkynyl radicals, amino radicals and sulfonic acid radicals and X is halogen.

2. The nickel plating solution of claim 1 which includes a wetting agent having the formula



wherein R<sub>4</sub> is an alkanoyl radical having 8 to 10 carbon atoms; R<sub>5</sub> is selected from the group consisting of hydrogen, aliphatic, alicyclic and aromatic radicals; R<sub>6</sub> is an aliphatic bridge containing from 1 to 5 carbon atoms and R<sub>7</sub> is selected from the group consisting of hydrogen and alkali metal.

3. The nickel plating solution of claim 2 wherein the wetting agent is present in amounts of 0.5 to 5 g/l. of solution.

4. The nickel plating solution of claim 1 which includes a hydroxy derivative of an aromatic sulfur compound as a sequestering agent.

5. The nickel plating solution of claim 4 wherein the hydroxy derivative of an aromatic sulfur compound is sodium tetrahydroxynaphthalene sulfonic acid.

6. The nickel plating solution of claim 4 wherein the hydroxy derivative of an aromatic sulfur compound is present in amounts of 0.1 to 5 g/l. of solution.

7. The nickel plating solution of claim 1 wherein the brightener is present in amounts of 0.01 to 10 mmol/l. of solution.

8. The nickel plating solution of claim 1 which includes as an additional brightener an aromatic sulfur compound.

9. The nickel plating solution of claim 8 wherein the additional brightener is sodium saccharate.

10. The nickel plating solution of claim 8 wherein the additional brightener is naphthalene trisulfonic acid.

11. An aqueous acid bath solution for electroplating nickel containing at least one nickel salt as a source of nickel which plating solution includes as first brightener a sufficient amount of a compound selected from the group consisting of compounds having the structural formula



and



wherein R, R<sub>1</sub>, R<sub>2</sub> and R<sub>3</sub> are selected from the group consisting of hydrogen, alkanyl, alkenyl and alkynyl radicals, hydroxy derivatives of said alkanyl, alkenyl and alkynyl radicals, amino radicals and sulfonic acid radicals and X is halogen.

12. The nickel plating solution of claim 11 which includes a wetting agent having the formula



wherein R<sub>4</sub> is an alkanoyl radical having 8 to 10 carbon atoms; R<sub>5</sub> is selected from the group consisting of hydrogen, aliphatic, alicyclic and aromatic radicals; R<sub>6</sub> is an aliphatic bridge containing from 1 to 5 carbon atoms and R<sub>7</sub> is selected from the group consisting of hydrogen and alkali metal.

13. The nickel plating solution of claim 12 wherein the wetting agent is present in amounts of 0.5 to 5 g/l. of solution.

14. The nickel plating solution of claim 11 which includes a hydroxy derivative of an aromatic sulfur compound as a sequestering agent.

15. The nickel plating solution of claim 14 wherein the hydroxy derivative of an aromatic sulfur compound is sodium tetrahydroxynaphthalene sulfonic acid.

16. The nickel plating solution of claim 14 wherein the hydroxy derivative of an aromatic sulfur compound is present in amounts of 0.1 to 5 g/l. of solution.

17. The nickel plating solution of claim 11 wherein said first brightener is present in amounts of 0.01 to 10 mmol/l. of solution.

18. The nickel plating solution of claim 11 which additionally includes as a second brightener an aromatic sulfur compound present in amounts of 0.1 to 30 g/l. of solution.

19. The nickel plating solution of claim 18 wherein said aromatic sulfur compound is sodium saccharate.

20. The process of producing nickel deposits of improved ductility and corrosion resistance characteristics on a metal base which comprises electrodepositing nickel from an aqueous acid bath containing nickel mainly in the form of a soluble inorganic salt, in the presence of a brightener selected from the group consisting of compounds having the structural formula



50

and



60

and



wherein R, R<sub>1</sub>, R<sub>2</sub> and R<sub>3</sub> are selected from the group consisting of hydrogen, alkanyl, alkenyl and alkynyl radicals, hydroxy derivatives of said alkanyl, alkenyl and alkynyl radicals, amino radicals and sulfonic acid radicals and X is halogen, said brightener being present in an amount sufficient to produce a bright nickel deposit.

21. The process of claim 20 wherein the brightener is present in amounts of 0.01 to 10 mmol/l. of solution.

22. The process of claim 20 wherein said bath includes an aromatic sulfur compound.

23. The process of claim 22 wherein said brightener is present in amounts of 0.05 to 5 mmol/l. of solution and said aromatic sulfur compound is present in amounts of 0.1 to 30 g/l. of solution.

24. The process of claim 20 wherein said bath includes a wetting agent having the formula



wherein  $R_4$  is an alkanoyl radical having 8 to 10 carbon atoms;  $R_5$  is selected from the group consisting of hydrogen, aliphatic, alicyclic and aromatic radicals;  $R_6$  is an aliphatic bridge containing from 1 to 5 carbon atoms and  $R_7$  is selected from the group consisting of hydrogen and alkali metal, said wetting agent being present in amounts of 0.5 to 5 g/l. of solution. 5

25. The process of claim 20 wherein said bath includes a hydroxy derivative of an aromatic sulfur compound as a sequestering agent. 15

26. The process of claim 25 wherein the hydroxy derivative of an aromatic sulfur compound is sodium tetrahydroxynaphthalene sulfonic acid.

## References Cited

## UNITED STATES PATENTS

|           |        |                     |              |
|-----------|--------|---------------------|--------------|
| 2,460,233 | 1/1949 | Morris et al. ----- | 260—332.1    |
| 2,504,099 | 4/1950 | Morris et al. ----- | 260—332.1    |
| 2,539,588 | 1/1951 | Moy -----           | 204—49       |
| 2,678,910 | 5/1954 | Brown -----         | 204—49       |
| 3,041,255 | 6/1962 | Passal et al. ----- | 204—49       |
| 3,098,793 | 7/1963 | Loev -----          | 260—332.1 XR |
| 3,130,135 | 4/1964 | Ericson -----       | 204—49       |
| 3,261,772 | 7/1966 | Ericson -----       | 204—49       |
| 3,306,912 | 2/1967 | Fritz et al. -----  | 260—332.1    |

HOWARD S. WILLIAMS, Primary Examiner.

G. KAPLAN, Assistant Examiner.